

# UNITED STATES PATENT OFFICE.

CLARENCE A. WHITMYRE, OF SCHENECTADY, NEW YORK, ASSIGNOR TO GENERAL ELECTRIC COMPANY, A CORPORATION OF NEW YORK.

## TREATING HIGH-SPEED STEEL.

1,359,851.

Specification of Letters Patent. Patented Nov. 23, 1920.

No Drawing.

Application filed August 2, 1919. Serial No. 314,968.

To all whom it may concern:

Be it known that I, CLARENCE A. WHITMYRE, a citizen of the United States, residing at Schenectady, county of Schenectady, 5 State of New York, have invented certain new and useful Improvements in Treating High-Speed Steel, of which the following is a specification.

The present invention relates to the heat 10 treatment of high speed alloy steel and particularly to the quenching of steel after having been heated to a high temperature in order to harden and temper the same.

It is the object of my invention to avoid 15 cracks in the hardened steel and to improve the quality of the steel.

Prior to my invention it has been customary to heat cutters and similar high speed steel tools to a high temperature and then 20 to quench them by cooling in a bath of oil or in an air blast. In accordance with my invention improved results are obtained by heating the high speed steel to a temperature of about 1275° to 1300° C. and then 25 quenching the heated steel at a temperature of about 600-650° C., preferably by contact with a bath of fused salt maintained at a desired temperature. In other words, I arrest the quenching temperature at 600-650° 30 C. to avoid the drastic effect of immediate cooling from 1300° C. to room temperature.

High speed steel, as distinguished from nickel steel, or carbon steel, is characterized by a high tungsten content. A typical high 35 speed steel contains besides iron the following: tungsten 13 to 15%; chromium 3.5 to 4.25%; carbon .55 to .70%; vanadium 1%; silicon 15 to 21%; manganese .20 to .40%; sulfur and phosphorus being kept 40 negligibly low.

When carrying out my invention the tool to be hardened is first slowly preheated to about 850° C. in any convenient way, say, for example, in an oil, gas or electric furnace in the usual well understood manner. 45 The tool is then heated from 850° C. as rapidly as is desired to 1300° C. in any suitable furnace. When the tool has reached the temperature of 1275° to 1300° C. it is 50 removed and immersed in a bath of fused salts maintained at a temperature of about 600-650° C. Any desired quenching bath, maintained at this temperature range, may

be used, but I prefer to employ a bath consisting of the chlorids of potassium, sodium, calcium and barium used in equal proportions by weight. When the high speed steel tool has attained the temperature of this quenching bath, it is removed and allowed to cool in the air. If desired, the hardened 60 tool may be subsequently heated or "drawn" to remove strains in the usual manner.

What I claim as new and desire to secure by Letters Patent of the United States, is,—

1. The method of hardening high speed 65 steel which consists in heating the steel to a temperature of about 1275° to 1300° C. and then quenching the same at temperature of about 600-650° C.

2. The method of quenching alloy steel 70 which consists in heating the steel to a temperature of about 1275° to 1300° C. and then reducing the temperature of said steel to about 600 to 650° C. by contact with a bath of fused salts.

3. The method of hardening tungsten 75 steel which consists in heating steel to a temperature of about 1275° to 1300° C. and then quenching the heated steel by contact with a bath of molten chlorids of potassium, sodium, calcium and barium in equal proportions by weight, said bath being heated to a temperature of about 600-650° C.

4. A quenching bath for high speed steel 85 consisting of the chlorids of potassium, sodium, calcium and barium in proportions adapted to cause said bath to be liquid at about 600 to 650° C.

5. A quenching bath for high speed steel 90 consisting of the chlorids of potassium, sodium, calcium and barium in equal proportions by weight.

6. The method of hardening steel tools 95 containing at least about 13% tungsten, which consists in slowly heating said tools to about 850° C., then rapidly raising the temperature of said tool to about 1300° C., thereupon quenching the heated tool in a bath of fused salts maintained at a temperature of about 600 to 650° C. and finally permitting said tool to cool in the air.

In witness whereof, I have hereunto set my hand this 1st day of August, 1919.

CLARENCE A. WHITMYRE.